

June 25, 1929.

L. R. MacKENZIE

1,718,863

IMPACT METHOD OF MAKING PAVEMENT

Filed Sept. 15, 1928

2 Sheets-Sheet 1

Fig. 1



Witness  
R. A. Rushey

Inventor  
"Leon R. MacKenzie"  
by Bair, Freeman & Sinclair  
Attorneys

June 25, 1929.

L. R. MacKENZIE

1,718,863

IMPACT METHOD OF MAKING PAVEMENT

Filed Sept. 15, 1928 2 Sheets-Sheet 2



Witness  
Dinton Read.

Inventor  
Leon R. MacKenzie  
by Bair, Freeman & Sinclair  
Attorneys

## UNITED STATES PATENT OFFICE.

LEON R. MACKENZIE, OF DES MOINES, IOWA.

## IMPACT METHOD OF MAKING PAVEMENT.

Application filed September 15, 1928. Serial No. 306,208.

The purpose of my invention is to provide a method for making a concrete pavement, which is as close in nature to hard natural stone as it is possible to secure.

5 It is the purpose of all constructors of concrete pavement to secure a pavement having as nearly as possible the structure, durability and permanence of hard natural stone. If it were possible to cut slabs of hard natural 10 stone, transport and lay them for paving, this would make the ideal hard surfaced pavement. Practically and economically, it has become necessary to crush the stone into relatively small particles, add cement, water 15 and fine particles, then mix together to form concrete, and lay the concrete. The concrete as ordinarily mixed and laid has many air voids and has considerable excess water content over the amount required for complete 20 hydration of the cement particles.

It is desirable to eliminate the voids, created by air and excess water content, in order to leave a finished product which is as dense and homogeneous as is possible to secure, consisting of hard rock aggregate driven into close relation with each other and properly bonded or cemented together by the cement 25 mortar contained therein.

In practical concrete paving construction, 30 for ease of transportation and handling, it is necessary that the proportion of mortar to stone be greater than it should be under ideal conditions. In pavements actually built the mortar in concrete is never as strong as the 35 hard rock aggregate itself.

Various methods have been employed tending toward the elimination of excess water and the air in the plastic concrete. What is probably the most common practice involves 40 the use of heavy tampers applied direct to the concrete that does up to a certain point compress the plastic mass, forcing out some excess water and air in parts of the structure. This method is successful only to a degree for the 45 reason that it is impossible to make the mass homogeneous throughout. The water and air are taken from the upper part of the slab to a shallow depth but they are not sufficiently removed from the lower part of the body.

50 Various methods for vibrating and agitating the concrete have been heretofore used, and by them a better result has been obtained than by heavy tamping alone.

So far as I know none of these methods, 55 however, have resulted in a concrete slab of

maximum and uniform density, strength and wear resisting qualities.

It is therefore my object to provide an economical method for making concrete pavement or the like, which will be free from numerous disadvantages to which methods heretofore used have been subject.

Another purpose is to provide such a method by which there may be constructed a concrete pavement with a minimum amount of 65 mortar content and a maximum amount of hard rock aggregate, properly compressed, so as to make as nearly as possible a synthetic rock having the homogeneous nature of a 70 monolithic hard rock slab.

It is a further purpose of my invention to provide such a process, which is mechanical, more rapid and more economical in operation than those heretofore employed.

Particularly it is my purpose to provide 75 such a method involving the use of direct vertical impacts imposed upon suitable grids or the like and thus conveyed to the plastic concrete for uniformly condensing the concrete in the shortest possible time and with 80 the greatest mechanical efficiency and for thus effecting more completely than has ever before been done the removal of excess water and air voids from the completed mass.

For the purpose of illustrating a practical 85 means for practising my method, I have shown drawings accompanying this application, in which:

Figure 1 is a perspective view of a section of pavement on which are grids and an impacting machine with which my invention 90 may be practised.

Figure 2 is a sectional view through the impacting machine.

Figure 3 is a vertical, sectional view of the 95 unbalanced, overweighted vertical piston and connected parts of the impacting machine taken on the line 3—3 of Figure 2; and

Figure 4 is a horizontal sectional view taken on the line 4—4 of Figure 2. 100

I shall now describe somewhat in detail the steps employed in the practice of my method.

I first mix concrete as usual, except that on account of the greater force of the impact to which the product is to be subjected and the direct vertical nature of the impact and the consequent complete subjection of the entire mass to the action of the repeated impacts, I am able to use substantially less of the cement mortar and a greater proportion of coarse 105

hard rock aggregate, than have hitherto been generally used in making concrete pavement.

For instance, I suggest a concrete mixture of substantially different proportions than 5 has heretofore been used and standardized for such purpose. Standardized concrete mixes all carry a volume of mortar in terms of percentage of volume of stone aggregate considerably in excess of 50%, whereas in the mix 10 I will use in my method, the volume of mortar in terms of percentage of the volume of stone aggregate can be less than 50%, in the completed pavement. The cement, fine and coarse aggregate in proper portions are mixed 15 with the addition of water in the usual way under prevailing standard requirements.

This concrete mix is then laid on the sub-grade in the ordinary way.

My method may be employed with or without 20 the use of added surfacing stone.

If surfacing stone is not used, an equivalent amount of coarse material of similar size is incorporated into the concrete mixture as it goes into the mixer drum. The concrete surface 25 is struck or leveled in the usual way after being placed on the prepared sub-grade.

If surfacing stone is used, there is placed on the plastic concrete after being leveled and before it is hardened a covering of hard 30 crushed stone of the kind acceptable in standard specifications having a maximum size of from one to three inches or preferably one to two and one-half inches, which will make a surface layer substantially one inch thick 35 when impacted into the solid mass.

I then lay grids or impact conveying units on the top stone or the prepared surface of the concrete. These units, in sections, are fitted together to furnish a supporting semi-rigid 40 surface on which the impacting machines can be moved freely from place to place. Likewise they serve the function of conveying the impact to the top stone and/or to the plastic concrete. They also serve as a restraining 45 medium for maintaining the surface being impacted in substantially uniformly level position, instead of permitting parts to be pressed down while other parts bulge up. They likewise serve a function in that they 50 hold the concrete in place between successive impacts by their own weight and the weight imposed upon them, so that upon the return or upward stroke of the impacting machine, the plastic material will not return to its condition 55 as it existed before the previous impact.

The next step in the practice of the method involves placing the impact machine upon the units and freely and independently moving it longitudinally of the pavement and also 60 diagonally in both directions across the pavement slab and operating it for imparting to the plastic concrete the successive direct downward impacts by which the ultimate desirable result is attained.

65 I shall now describe an apparatus which

may be used in the practice of my method and shall then explain some of the important features and advantages of the apparatus and method.

The impact conveying units employed may 70 be such as those described in my co-pending application, filed September 8, 1928, Serial No. 304,788.

Generally they are composed of light metal, such as aluminum, or gum wood or other light 75 material or a combination of metal and wood. They may have a series of properly spaced cleats, indicated in the drawings by the reference numeral 10, of true surfaces. Their upper and lower surfaces normally rest in parallel 80 horizontal planes. The cleats of each unit are held in place therein by the rods 12 extending through the cleats the full length of the unit. The ends of the rods are threaded to receive nuts 14, which are used with lock 85 washers 16. The nuts are thus adjustable for keeping the rods taut and holding the units to shape while allowing sufficient flexibility for properly carrying out my method. Metal or wood spacing blocks 18 are arranged on the 90 rods 12 between the successive cleats 10.

The units may be made with the cleats running longitudinally of the pavement, with the tie rods arranged transversely as explained in my co-pending application. 95

The drawings here are simply illustrative. Other forms of units may be used. It is important that the area bearing on the pavement be at least twice the area of the openings which permit the escape of air and excess 100 water from the concrete. Such openings also provide free visual observation of the mass worked upon and the condition thereof.

The impacting machine comprises a frame 19 supported on rollers and/or wheels 22, 105 adapted to travel freely and independently over the grids. On the frame is a vertically reciprocable device such for instance as the piston 28 forming part of an internal combustion engine having the cylinder 30, fly 110 wheels 32 and other usual operative mechanisms. The engine is in balance, as per standard construction, except for the weight of the piston which is preferably more than double that of the ordinary piston for an engine of similar bore and horse power, (see Figures 2, 3 and 4). 115

The frame 19 has the handles 34 by which an operator may move the machine from place to place. The throttle control 36 is accessible for controlling fuel feed from the handles for thus regulating the speed of the piston and consequently controlling the force of the impact. 120

The impacting desired may be secured by means of a vertically reciprocating member, other than the engine piston, driven from the engine or by a separate motor of the electric type or otherwise, so long as the driving and driven mechanisms are properly attached to 125 130

a mobile frame and produce downward vertical impacts through the frame and through the units to the concrete.

I shall now refer in greater detail to some of the steps of the method and to its advantages.

After the impacting of each section of pavement covered by the units has been carried out, the units are lifted and moved forward from one-half to three-quarters of their length and relaid without in any way disturbing the concrete surface previously established. The rear parts of the units then rest on portions of the concrete that have been impacted and the front portions on unimpacted concrete.

The impacting operation is repeated on the units as thus advanced. This cycle of operation is carried on for all the pavement laid.

After the impacting has been completed and the units advanced, the impacted concrete is left with shallow mortar ridges on the surface. These mortar ridges are then leveled and smoothed out and the mortar evenly distributed over the entire pavement surface.

The pavement surface is then finished by bolts, floats or the like in the usual manner for concrete pavements.

An important feature of the impacts produced in the practice of this method lies in the fact that they are at all times delivered direct and vertical and in a downward direction without loss by being diverted to other directions or being dissipated for other purposes. Another important feature of these impacts is the fact that no part of the impact is lost as is the case with ordinary concrete pavement finishing machines in the use of which, due to the fact that the weight of the tamping devices is carried upon the side forms or curbing, only a small part of the impact created by such machines is actually exerted upon the concrete itself. These other types of concrete pavement tamping and finishing machines actually act as a bridge over the concrete and furnish no sustained pressure or weight to the mass after each successive blow is imparted, hence the action on the concrete is on the surface only and for the depth of the blow given.

Still another important feature of this method is the flexibility of operation. Individual batches of concrete constituting the plastic mass vary somewhat in consistency and general makeup. For that reason different areas of the pavement surface will require longer and more vigorous treatment to bring them to the same condition as other parts of the surface more easily worked. It will thus be seen that the impact machine must be readily movable on and independently of the grids or conveying units for comparatively short distances in all directions as the condition of the plastic material may require, and it must be possible to apply the variable impact force over a limited area for

a long or short time as conditions may require.

A further important feature is the fact that the impact force may be greatly increased or decreased at will by merely increasing and decreasing the speed of the reciprocating member. Such variation is required by the variations in different batches of concrete in different parts of the pavement mass.

Thus an important feature of the impact process is the ability to apply variable impact forces readily over any limited areas for variable lengths of time as the variations in the concrete may require.

On account of the flexibility of the process, I insure certainty and uniformity in its practice.

The weight of the impact machine operating over the grids, together with the subjecting of the concrete to the successive vertical impacts of the machine will condense to its full depth the mass of concrete and if top stone is used will force it into the mass.

I find that there are substantial advantages in using a vertically reciprocating impact machine over a vibrating machine of the rotary type using un-balanced fly wheels or the like.

The use of the vertical stroke machine has less tendency to cause the units to travel longitudinally and laterally on the concrete. This is true because it gives the full force of the stroke in a direct line instead of having a glancing or shoving action. I thus effect an economy of power.

I find that the result of removing surplus water and air is more quickly and thoroughly secured by the vertical impacts than by rotary vibration machines. In part this is due to the fact that there is a tendency on the part of rotary machines to push the grids horizontally from their proper place. Consequently the units to some extent tend to pull the top surface of the concrete mass horizontally. This tends to pull the component parts of the pavement apart and counteracts that condensing and packing of the mass, which is the primary object in view. Such tendencies are avoided by my method.

For the same reason, there is less tendency for the vertical stroke machine to rock the grids and thus cause inequalities in the surface of the concrete pavement.

The result, which it is desired to accomplish is the elimination of the air voids and excess water in the concrete mixture, thereby condensing the mass and at the same time maintaining a true surface contour. With the successive impacts, the air is forced out, and the excess water comes to the surface and flows off between the cleats or through the openings of the units. The compression of the layer of concrete is accomplished much more quickly with a vertical stroke machine.

I find that the vertical type impact ma-

chine can be of less bulk and weight and still secure a better condensing result in quicker time.

Furthermore, because of the direct and heavier stroke delivered by the impact machine than is procurable with the rotary or vibrating type of machine, fewer blows are necessary and there is an economy in wear on the parts as well as of time consumed:

10 More important, than this advantage is the fact that a better and more uniform product is secured. This is the only method of which I am aware by which the voids in the concrete can be practically entirely eliminated.

Where the impact is by direct vertical action of the machine, and is thus imposed through the grids to the concrete, there is not only an increase in the speed of operation, but 20 also there is insured delivery of the entire impact force developed. This force is sufficient in amount to eliminate excess water and air voids, not only from the upper portions of the pavement mass, but from the entire lower 25 part thereof, so that when the product is completed by this method, the lower part of the pavement mass as well as the upper part becomes a homogeneous structure with a maximum of hard rock aggregate and a minimum 30 of mortar.

By using the method here employed, less mortar is put into the mix originally than it has been commercially possible to successfully operate with heretofore, and I find that there 35 is produced by my method a monolithic structure in which the rock aggregate particles are crowded so closely together that there is between them only a film of the binding mortar or cement.

40 There is thus attained the effect of a monolith of stone particles closely crowded together and bonded by thin layers of cement mortar into a slab, approaching as nearly as possible in its composition and strength and 45 wearing qualities, high grade natural stone in its original condition.

In addition to the fact that the impact method eliminates more excess water and air voids throughout the mass than other methods and devices have heretofore been able to 50 eliminate, I find that the impact method causes a change in the physical action of the cement used in the concrete. Portland cement is made from limestone, clay and certain other materials. The material is 55 burned, fused, and then ground very fine with the addition of a small amount of gypsum, which is for regulating the setting time or hardening time required for the cement, 60 after it is mixed with water. Cement is thus dehydrated and when mixed with water will 65 harden into a substance somewhat like stone. When water is added, changes take place in the physical and chemical structure of the cement particles.

I find that the use of the impact method applied to the concrete after it has been put into place from the mixer accomplishes two purposes not heretofore accomplished in ordinary concrete paving practice.

70 In the first place, it is equivalent to a re-mixing action on the concrete. During the discharge of the concrete from the mixer drum and the handling process, the concrete materials tend to segregate somewhat. The 75 application of the impact method tends to restore the original condition of the concrete as in the drum at the end of the mixing period and before being discharged. Each cement particle in the mass is thus given 80 ready access to the required amount of water for hydration and the formation of the cement crystals which is necessary to the binding properties of cement mortar. Thus hydration of a much larger percentage of the 85 cement particles than usual is accomplished, and the more complete hydration of all particles is facilitated and increased.

89 In the second place, by the use of the impact method prior to the hardening or setting process of the cement, certain changes occur in the form of the crystal, resulting in a different crystalline structure having a 90 higher cementing or binding property.

95 One of the results of the chemical and physical changes taking place is the formation of a definite and characteristic crystalline form in much the same way as snowflakes take a definite and characteristic form. Under the impact method this crystalline 100 form is different than usually secured, and this different form is also distinctly characteristic of impacted concrete when the hydration process is fully completed without interruption.

105 There thus results from the use of my method a more complete crystallization and a different and better crystallization of the cement.

110 Thus by the use of this method, there is secured a better product.

115 1st. Because the impacted concrete is more uniformly dense and therefore stronger, because I am enabled to use a higher percentage of the strongest element, to-wit, the coarse aggregate or hard stone in the mass.

120 2d. The density and consequently the strength of the resultant product is more uniform throughout the mass than where any other method known to me is used.

125 3d. The density and strength of the mortar consisting of cement, sand and water is also increased because of the more complete hydration and crystallization of the cement particles and of the different crystallization.

130 I have also determined by experiment that where this method is used, the concrete not only reaches a higher ultimate strength, but it acquires a relatively high percentage of its ultimate strength at a much earlier

stage than can be secured with any other process of which I am aware, and therefore is usable at a much earlier date than ordinary concrete.

5 By the use of the term "coarse aggregate" in my claims, I would include gravel pebbles, steel slag, crushed rock or other similar materials of proper size and structural qualities as ordinarily used in or adapted 10 to meet the requirements of pavement or other concrete construction.

Nor do I desire to limit myself to the use 15 of my method for pavements, but I intend to cover it for any concrete slab construction, 15 subject to abrasion or wherein the factor of dense concrete is a requisite.

I claim as my invention:

1. A method of making concrete pavement, comprising placing on a sub-grade a mass 20 of plastic pre-mixed concrete mortar and coarse aggregate in such proportions that the loose measured volume of coarse aggregate shall exceed by one hundred percentum or more the volume of mortar in the finished 25 pavement, placing on the mass while still plastic a plurality of grids, subjecting each of the consequently variable portions of the mass to constant pressure and to a succession of direct downward vertical impacts, regulated 30 as to force and as to location on the units, and for the proper length of time, to force the excess water and air from such portion throughout its full depth for thus forming a resultant pavement of maximum density 35 and substantially uniform composition.

2. A method of making concrete pavement, comprising placing on a sub-grade a mass of plastic concrete mortar and coarse aggregate, and then while the mass is still 40 plastic subjecting each consequently variable portion thereof to continued vertically downward pressure and repeated vertically directed downward impacts regulated as to force and as to location and for the proper

length of time to force upwardly the excess 45 water and air from each such portion for thus forming a resultant pavement of maximum density and substantially uniform composition.

3. A method of condensing concrete comprising placing on a suitable base a mass of plastic concrete, which varies in plasticity in different portions, then while the mass is still plastic, placing thereon impact conveying units wholly supported by the mass, then 50 subjecting the units while stationary to continued pressure and to repeated impacts imparted in vertical downward direction only and varying the location of application of the impacts and pressure on the conveying units, 55 and also varying the force, rapidity and duration of the impacts, as required by the variable plastic conditions of the various portions of the mass until the entire mass is compacted to 60 uniform density. 65

4. A method of condensing concrete consisting of placing on a suitable base a mass of plastic concrete, then while the mass is still plastic, placing thereon grating members through which the mass is discernible, then 70 placing on the grating members an impacting machine having a frame movable on the grating members and having parts arranged to deliver vertical blows to its frame, and then operating said machine on said grating members 75 to apply continued pressure and also to impart repeated vertical impacts through the machine frame and through said grating members, in a downward direction only, to the underlying mass, and regulating the force 80 of said impacts and the position of the impacting machine on the grating members as required by the inherently variable plastic conditions of the various portions of the mass 85 as disclosed through said grating members, until the entire mass is compacted to uniform density. 85

LEON R. MACKENZIE.